# EUROPEAN PATENT SPECIFICATION

(11) **EP 2 272 645 B1**
(45) Date of publication and mention of the grant of the patent: **02.09.2015**
(21) Application number: 10006901.2
(22) Date of filing: 05.07.2010
(51) Int. Cl.: B28B 11/00, B28B 11/08, B28B 11/18, B28B 11/24

(54) **Method for decorating ceramic products**
Verfahren zum dekorieren keramische Produkte
Méthode de décoration de produits céramiques

(30) Priority: 03.07.2009 IT MO20090175
(43) Date of publication of application: 12.01.2011
(73) Proprietor: SITI - B&T Group S.p.A., 41043 Modena (MO) (IT)
(72) Inventor: Tarozzi, Fausto, 41043 Formigine (Modena) (IT)
(74) Representative: Bergamini, Silvio

(56) References cited:
- EP-A1- 0 386 422
- EP-A2- 0 242 503
- EP-A2- 1 101 585
- DE-C1- 3 822 653
- US-A- 3 268 637

## Description

### Field of the invention

The present invention relates to a decorating method for decorating ceramic handmade products, such as tiles and slabs obtained by extrusion of a ceramic mixture.

### Background art

The prior art method for decorating ceramic handmade products, such as tiles and slabs, includes the steps of extruding a substantially continuous ribbon of a ceramic mixture in a plastic state, and later transversely cutting the ribbon to predetermined sizes, to obtain plastic and raw tiles and slabs.

The transverse cutting step is followed by a step in which the cut pieces so obtained are dried, and by a later step in which the surfaces designed to be exposed to view are decorated.

A variety of decoration techniques are available, e.g. including application of multicolored powder glaze on the surfaces of the raw pieces, or application of silk-screen prints using rotating devices that transfer the patterns formed by intaglio printing processes and suitably filled with inks and glazes, by tangential contact, i.e. by rolling on the surfaces to be decorated without appreciably slipping thereon.

Upon completion of the decoration step, the handmade products are introduced into a firing kiln, which stabilizes them and makes the decorations inseparable from the surfaces on which they have been applied.

This prior art suffers from the drawback that, upon firing, the handmade products obtained by extrusion are likely to be exposed to shrinkage, to different extents from one point to another, which are caused both by internal tensions generated in the extruded ribbon during extrusion through the dies, and by the moisture content in the mixture, which is not consistent throughout it.

Such shrinkage during cooking cause warping in the products, which lose their planarity: namely, the corners of the products tend to raise relative to their central area, whereas the sides perpendicular to the direction of extrusion bend and form a concave profile: such deformation requires the products to undergo a grinding treatment after firing.

Nevertheless, such treatment may cause damages to the decorations applied on the exposed faces of the products.

A further drawback is that the material removed during grinding cannot be recovered and reintroduced into the production cycle, as it has already been fired.

Another drawback is that this removed material mixes with the water that is used to cool the grinding wheels during the abrading action thereof.

Therefore, this water needs purification, by separation from the solid material mixed therewith, with the removed material being placed in settling tanks for gravity separation of solid parts and water: after purification, such water is reintroduced into the production cycle, whereas the solid part is pressed to obtain wet blocks to be carried and disposed of in landfills.

A further drawback is that, due to the plasticity of the extruded raw ceramic materials, the decorating glazes hardly penetrate them and tend to remain at their surfaces, thereby preventing, in certain cases, the final grinding step.

Yet another drawback is that, due to ceramic material saving requirements in product manufacture, products are required to be thinner and thinner, and handling of these thin products in the raw and plastic state is problematic, due to their tendency to spontaneous deformation.

US 3268637-A1 describes a decorating method according to the preamble of claim 1.

### Disclosure of the invention

One object of the invention is to improve the state of the art.

Another object of the invention is to provide a decorating method for decorating ceramic handmade products that allows the ceramic handmade products to be ground by a smoothing step, without damaging the decorations.

A further object of the invention is to provide a decorating method for decorating ceramic handmade products that allows recovery of the ceramic materials removed during the smoothing step and reintroduction thereof into the production cycle, without requiring any filtering and particulate matter removal equipment.

Yet another object of the invention is to provide a decorating method for decorating ceramic handmade products that allows handling of ceramic handmade products in a raw state without causing deformation thereof.

The invention relates to a decorating method for decorating ceramic handmade products as defined in claim 1.

Therefore, the invention provides the following advantages:
a) Obtaining extruded and decorated ceramic handmade products, that may be flattened by a smoothing step, with the latter causing no damage to decorations;
b) Improving the bond between the decorating lacquers and the handmade products, by promoting deep penetration of the products by the lacquers;
c) Saving ceramic material by recovering the material removed during the grinding step to flatten the handmade products and reintroducing it into the production cycle;
d) Obtaining thinner ceramic products than in the prior art, with considerable raw material savings.

Furthermore, the decorating method for decorating ceramic handmade products may be also used on existing and operating decorating plants, without requiring particularly difficult and costly structural adaptations.

### Brief description of the drawings

Further characteristics and advantages of the invention will be more apparent from the detailed description of a few preferred, non-exclusive embodiments of a decorating method for decorating ceramic handmade products according to the invention, which are described as non-limiting examples with the help of the annexed drawing, in which:
FIG. 1 is a block diagram of the operating steps of a prior art decorating method for decorating ceramic handmade products;
FIG. 2 is a block diagram of the operating steps of a decorating method for decorating ceramic handmade products according to the invention.

### Detailed description of a preferred embodiment

Referring to Figure 1, the prior art decorating method for decorating ceramic handmade products obtained by extrusion of ceramic material in a plastic state, includes an extrusion step, designated by numeral 1, in which a laminar ceramic ribbon is extruded, raw ceramic handmade products in a plastic state being obtained from such ribbon.

The step of extruding and obtaining raw ceramic handmade products in a plastic step is followed by a step, designated by numeral 2, in which the ceramic handmade products are dried, a step, designated by numeral 3, in which the in sight surfaces of the ceramic products are decorated, a step, designated by numeral 4, in which the decorated ceramic products are fired and a final step in which the fired ceramic products with planarity defects are ground.

According to the invention and referring to Figure 2, a step of extruding and obtaining raw ceramic handmade products in a plastic state and with predetermined size is included and designated by numeral 101, to differentiate it from the previous figure.

Numeral 102 designates a later step of drying the raw ceramic handmade products, in which removal of most of the moisture in the raw ceramic products by evaporation after extrusion makes such products more compact and cohesive, substantially free of their initial plasticity: this provides bodies whose mechanical strength allows handling thereof without causing deformation.

Numeral 103 designates a later step in which the planarity of the top surfaces of the ceramic handmade products, which are designed to be the exposed surfaces thereof, is restored by smoothing.

In addition to restoring the planarity of the ceramic product surfaces, this smoothing step 103 also adds porosity to these surfaces, and hence makes them more prone to absorb and deeply embed the lacquers that are used to make the decorations, which are sprayed in nebulized, atomized form by spraying devices.

In this smoothing step 103, the ceramic material removed from the smoothed surfaces may be, and actually is, recovered after suitable filtering, e.g. using bag filters, and reintroduced into the production cycle because it has not been fired yet, and hence has not irreversibly changed its state.

Numeral 104 designates a later step in which the in sight surfaces of ceramic handmade products that have been dried and ground in the smoothing step 103 are decorated.

This decorating step is carried out using the so-called ink-jet technique, in which a series of ejecting nozzles of a decorating plant spray colored nebulized lacquers on the in sight surfaces of the handmade products to form decorations thereon.

The decorating step 104 is followed by a final firing step, in which the decorated handmade products are fired for the decorations to be stabilized and molecularly bonded to the handmade products.

## Claims

1. A decorating method suitable for decorating handmade ceramic products, comprising:
- extruding a substantially laminar ribbon of ceramic material in a raw and plastic condition according to an extruding direction;
- obtaining raw and plastic handmade products from said ribbon;
- drying said raw and plastic handmade products obtaining raw products having cohesive bodies;
- decorating in sight surfaces of said cohesive bodies, obtaining raw and decorated handmade products; and
- firing said raw and decorated handmade products, **characterized in that** after said drying and before said decorating, grinding defects of said in sight surfaces of said cohesive bodies.

2. A decorating method according to claim 1, wherein said decorating comprises decorating by ink-jets.

3. A decorating method according to claim 1 or 3, wherein said grinding further comprises recycling ceramic material removed by said grinding.

4. A decorating method according to claim 1, wherein said obtaining step comprises cutting said ribbon according to fixed dimensions and directions.

## Patentansprüche

1. Ein Verfahren zum Verzieren, das geeignet ist zur Verzierung handgefertigter, keramischer Erzeugnisse, das umfasst:
- Ausziehen eines im Wesentlichen flächigen Bandes aus keramischem Material in einem rohen und verformbaren Zustand gemäß einer Ausziehrichtung,
- Erhalten von rohen und plastischen, handgefertigten Erzeugnissen aus diesem Band,
- Trocknen dieser rohen und plastischen, handgefertigten Erzeugnisse, um rohe Erzeugnisse mit kohäsiven Körpern zu erhalten,
- Verzieren sichtbarer Oberflächen der kohäsiven Körper, um rohe und verzierte, handgefertigte Erzeugnisse zu erhalten, und
- Brennen der rohen und verzierten, handgefertigten Erzeugnisse,
**gekennzeichnet durch** Schleifen von Fehlern an den sichtbaren Oberflächen der kohäsiven Körper nach dem Trocknen und vor dem Verzieren.

2. Ein Verfahren zum Verzieren gemäß Anspruch 1, wobei das Verzieren verzieren mittels Tintenstrahlen umfasst.

3. Ein Verfahren zum Verzieren gemäß Anspruch 1 oder 3, wobei das Schleifen zudem das Wiederverwenden von keramischen Material umfasst, das mittels Schleifen entfernt wurde.

4. Ein Verfahren zum Verzieren gemäß Anspruch 1, wobei der Schritt des Erhaltens schneiden des Bandes gemäß festen Abmessungen und Richtungen umfasst.

## Revendications

1. Procédé de décoration de produits céramiques faits à la main, comprenant:
- l'extrusion d'une bande essentiellement laminaire de matière céramique en condition brute et plastique dans une direction d'extrusion ;
- l'obtention de produits faits à la main bruts et plastiques de ladite bande ;
- le séchage desdits produits faits à la main bruts et plastiques pour obtenir des produits bruts ayant des corps cohésifs ;
- la décoration des surfaces exposées desdits corps cohésifs, pour obtenir des produits fais à la main bruts et décorés ; et
- la cuisson desdits produits faits à la main bruts et décorés, **caractérisé en ce qu'**après ledit séchage et avant ladite décoration, il comporte la rectification des défauts desdites surfaces exposées desdits corps cohésifs.

2. Procédé de décoration selon la revendication 1, dans lequel ladite décoration comprend une décoration par des jets d'encre.

3. Procédé de décoration selon la revendication 1 ou 3, dans lequel ladite rectification comprend le recyclage de la matière céramique enlevée par ladite étape de rectifier.

4. Procédé de décoration selon la revendication 1, dans lequel ladite obtention comprend la coupe de ladite bande selon des dimensions et des directions fixes.
